

## UNITED STATES PATENT OFFICE

ADOLPH LIONEL BURLIN, OF LONDON, ENGLAND

## TREATMENT OF WASTE SPUN OR WOVEN TEXTILE MATERIAL

No Drawing. Application filed October 26, 1929, Serial No. 402,810, and in Great Britain November 2, 1928.

This invention relates to the treatment of waste spun or woven material arising in textile works, garment factories or the like or which are obtained from rag merchants and has for its object to provide an improved method of treating such waste containing silk, wool, artificial silk, cotton or other fibres in order to obtain therefrom fibres adapted to be respun into yarns with or without the addition of virgin fibre.

The invention is mainly concerned with the treatment of waste spun or woven material containing artificial silk in connection with which the known processes of treating the same have resulted in crude and unsatisfactory results in that the original lustre of the artificial silk is lost and spinners have experienced difficulty in treating the carded artificial silk fibre.

According to the present invention, the waste is subjected to the action of aqueous detergents and before or after treatment in an opening carder is treated with a weak acid, for instance boric acid, and dextrine or soluble starch or the like.

After being subjected to the action of a detergent the textile waste may be treated with a solution of a neutral salt, for instance, sodium sulphate.

Further, in accordance with the invention, if the waste treated consists of or contains a material proportion of artificial silk the same is advantageously subjected to the action of a solution containing acid ammonium phosphate in addition to boric acid.

If the waste contains cotton fibre which it is desired to return in an uninjured state the above-mentioned treatment with acid ammonium phosphate should however be omitted.

Normally the material which will be treated in accordance with the invention will be received in the form of bales which will be opened up and may be disinfected, for instance, by the aid of formaldehyde.

The waste may also be beaten to remove dust prior to treatment with a detergent.

The order of the mechanical and other treatments to which the material is subjected may be varied within certain limits. For in-

stance, the waste material after treatment to remove dust and washing with a detergent may be treated with a solution of sodium sulphate and dried, the washed and dried material being then cut up into suitable sized fragments which by means of machines of generally known character are disintegrated or opened up, the fibrous material obtained being carded and subjected to the action of a solution containing essentially a weak acid, for instance boric acid, and dextrine or soluble starch.

As above indicated if the waste treated consists wholly or mainly of artificial silk, silk or wool but free from cotton, the solution employed in this stage will contain also ammonium phosphate.

For instance, when treating cotton free waste containing artificial silk, silk or wool in accordance with the invention, the solution may contain boric acid, acid ammonium phosphate and soluble starch in the relative proportions 2:2:1 and in a concentration of one gram per litre.

In treating, for instance, waste rags consisting wholly or mainly of artificial silk the rags may be freed from dust or dirt by mechanical processes, sorted with the aid, for instance, of an endless belt conveyor, cut up into pieces of 2 or 3 inches in length by a rag-cutting machine, such for instance as is used in a fine paper factory.

The cut rags are then opened up by treatment with an opening carding machine, washed in warm water with the addition of suitable detergents, for instance, soap flakes, dyed if necessary, to obtain a uniformly coloured product, and dipped into a solution containing a weak acid and a proportion of soluble starch.

This dipping may be carried out by treating the fibre with a solution containing 1 oz. of boric acid and  $\frac{1}{8}$  oz. soluble starch to each 10 gallons of cold water and as indicated this solution may also contain acid ammonium phosphate.

After treatment in such a solution for a relatively brief period, for example, ten minutes, the waste is taken out, lightly pressed and

dried, the drying operation being carried out, for instance, in a wool drying machine.

The finishing of the fibres may be effected on a fine finisher carder and coiler before reaching the condenser, whereby slivers ready for spinning are produced.

Yarns of fine counts can be spun from the finished fibres on a cotton spinning machine while the coarser yarns may be spun on worsted spinning machines and in the spun condition the yarns may be used for different purposes either alone or in association with real silk, cotton, wool or linen so as to obtain products of high or low lustre.

As will be understood the above description is furnished for the purpose of describing the nature of the invention and certain detailed methods of carrying the invention into effect. Various changes, however, may be made in the treatment to which the waste or the fibres are subjected without exceeding the scope of the present application.

Having now described my invention what I claim as new and desire to secure by Letters Patent is:—

1. The process of treating waste spun or woven material containing artificial silk which comprises subjecting the material to the action of aqueous detergents and thereafter treating the same with an acid body including boric acid, and a carbohydrate.

2. The process of treating waste spun or woven material containing artificial silk which comprises subjecting the material to the action of aqueous detergents subsequently treating the same with a neutral salt and thereafter subjecting it to treatment with an acid body including boric acid and a carbohydrate.

3. The process of treating waste spun or woven material containing artificial silk which comprises subjecting the material to the action of aqueous detergents and thereafter treating the same with boric acid, acid ammonium phosphate and soluble starch.

4. The process of treating waste spun or woven material containing artificial silk which comprises subjecting the material to the action of aqueous detergents subsequently treating the same with a neutral salt and thereafter subjecting it to treatment with boric acid, acid ammonium phosphate and soluble starch.

5. The process of treating waste spun or woven material containing artificial silk which comprises subjecting the material to the action of aqueous detergents and thereafter treating the same with a solution containing .4 gram per litre boric acid, .4 gram per litre acid ammonium phosphate, and .2 gram per litre of soluble starch.

6. The process of treating waste spun or woven material containing artificial silk which comprises subjecting the material to the action of aqueous detergents, subse-

quently treating the same with a neutral salt and thereafter treating it with a solution containing .4 gram per litre boric acid, .4 gram per litre acid ammonium phosphate, and .2 gram per litre soluble starch.

7. The process of treating waste spun or woven material containing artificial silk which comprises subjecting the material to the action of a solution of soap flakes in warm water dyed to obtain a uniformly coloured product and thereafter treating the same with an acid body including boric acid and a carbohydrate.

8. The process of treating waste spun or woven material containing artificial silk which comprises subjecting the same to the action of an aqueous solution of soap flakes in warm water dyed to obtain a uniformly coloured product, subsequently treating the same with a neutral salt and thereafter subjecting it to treatment with an acid body including boric acid and a carbohydrate.

9. The process of treating waste spun or woven material containing artificial silk which comprises subjecting the material to the action of a solution of soap flakes in warm water dyed to obtain a uniformly coloured product and thereafter subjecting it to treatment with boric acid, acid ammonium phosphate and soluble starch.

10. The process of treating waste spun or woven material containing artificial silk which comprises subjecting the material to the action of a solution of soap flakes in warm water dyed to obtain a uniformly coloured product, subsequently treating the same with a neutral salt and thereafter subjecting it to treatment with boric acid, acid ammonium phosphate and soluble starch.

11. The process of treating waste spun or woven material containing artificial silk which comprises subjecting the material to the action of a solution of soap flakes in warm water dyed to obtain a uniformly coloured product, subsequently treating the same with a neutral salt and thereafter subjecting it to treatment with a solution containing .4 gram per litre boric acid, .4 gram per litre acid ammonium phosphate and .2 gram per litre soluble starch.

12. The process of treating waste spun or woven material containing artificial silk which comprises subjecting the material to the action of a solution of soap flakes in warm water dyed to obtain a uniformly coloured product and thereafter subjecting it to treatment with a solution containing .4 gram per litre boric acid, .4 gram per litre acid ammonium phosphate and .2 gram per litre soluble starch.

In testimony whereof I have signed my name to this specification.

ADOLPH LIONEL BURLIN.